# EUROPEAN PATENT APPLICATION

(11) **EP 0 498 229 A1**
(43) Date of publication of application: **12.08.1992**
(21) Application number: 92101129.2
(22) Date of filing: 24.01.1992
(51) Int. Cl.: B44C 1/24, B44D 2/00, B44D 5/00

(54) **A method for the painting of a panel, a pulp sheet or a pulp web**

(30) Priority: 08.02.1991 FI 910618
(71) Applicant: FINNISH FIBREBOARD LTD., SF-28800 Pori (FI)
(72) Inventor: Saarinen, Esa, FI-28400 Ulvila (FI); Varjus, Kirsi, FI-28300 Pori (FI)
(74) Representative: Weitzel, Wolfgang, Dr.-Ing.

(57) **Abstract**

The invention relates to a method for producing a three-dimensional surface effect on a panel, a pulp sheet or a pulp web, in which method a coloring substance or coloring substances is/are sprayed from an angle of less than 90 degrees onto the surface of a rough-surfaced or relief-patterned pulp sheet or pulp web, whereby a three-dimensional effect is produced. The pulp sheet or pulp web is pressed after the spraying.

## Description

The invention relates to a method for producing a three-dimensional surface effect on a panel, a pulp sheet or a pulp web, in which method a coloring substance or coloring substances is/are sprayed onto the surface of a rough-surfaced or relief-patterned panel, pulp sheet or pulp web. Thereafter the pulp sheet or pulp web is pressed flat, or a relief pattern is formed on its surface in connection with the pressing. Thus a three-dimensional effect is produced.

Previously the painting of panels or sheets was not carried out until on the surface of an otherwise completed panel or sheet, on a separate painting line. Thereby panels which were single-colored or had simple patterns were obtained. In another method according to the state of the art, the pattern has been obtained on the surface of a completed panel by coating the panel with a thin paper on which the desired pattern has been printed.

The current methods of painting and coating panels are expensive and cumbersome, and the paints and papers required for them also cause considerable costs. Furthermore, these prior-known methods require trained personnel. Three-dimensional patterns cannot be painted on a conventional painting line; they should be hand painted by a professional painter.

The method according to the present invention deviates completely from previous methods, and it provides a crucial improvement over the methods described above. In the method according to the invention, a coloring substance or coloring substances is/are sprayed onto the surface of a pulp sheet or a pulp web from an angle of less than 90 degrees, before it is pressed, but after a relief pattern has first been produced on the surface of the pulp sheet or pulp web by using, for example, a roll or an upper wire unit, or the surface of the sheet has otherwise been left rough. In connection with the pressing, it is still possible to form on the surface of the pulp sheet or pulp web a relief pattern which repeats the painted pattern or deviates from it. In one alternative embodiment of the invention, a completed relief-patterned panel is painted by spraying a coloring substance or coloring substances onto the panel surface from one or several directions. The composition of the coloring substance is important in terms of the invention, since because of this the coloring substance will not adhere to the polish patterns of the press during the pressing.

The essential characteristics of the invention are presented in the accompanying claims.

The economy of the method according to the invention can be deemed to be one of its important advantages. It is not necessary to have a separate painting line for the painting; the painting can be carried out in connection with the normal manufacture of the panel. The pattern and colors can also be varied easily. Painting of good quality is obtained, in which case the panels, when placed next to each other, do not have visually detectable differences in tone or otherwise. In the method according to the invention it is possible to use, for example, a paint composition in which the principal component is a chalk slurry. Chalk slurry is economical, and it ensures that the coloring substance will not adhere to the polish patterns of the press during the pressing. Other paint compositions can also be used.

By means of the method and coloring substance composition according to the invention, the healthiness of the working environment can also be crucially improved, since a conventional painting line is not required, and thus the hazards due to solvents and vapors are avoided.

A panel produced by the method according to the invention may be the final product, or it may further be given a lacquer finish.

The invention is described below in detail, with reference to the accompanying figure, in which the steps of the method are depicted schematically.

The figure shows a pulp sheet 1, on which relief patterning is produced by means of a roll 2. The relief patterns may also be produced by some other method, for example by using an upper wire unit, in which case the pattern of the wire is left in the sheet. The sheet may also be left without a relief pattern, since before the pressing a sheet always has some roughness, which will be made visible by the coloring of the sheet when the painting method according to the invention is used. After a relief pattern has been produced by some method, the sheet is conveyed to the spraying lines 3 and 4, in which the pulp sheet is sprayed with different colors from different directions. When the coloring substance is sprayed laterally from an angle of less than 90 degrees, the shaded sides of the relief patterns in the pulp sheet are left uncolored. There may also be only one spraying line, in which case the color of the pulp will remain the base color of the sheet. There may also be more than two painting lines, and sprays for different colors may be installed in one and the same line. At a point after the painting line/lines, wax is sprayed onto the surface of the pulp sheet in a spraying line 5, before the sheet is conveyed to the press. After the pressing the colored relief patterns of the pulp sheet will appear three-dimensional in the flat surface.

In one embodiment of the invention, the pulp sheet is first pressed in a press, whereby a relief pattern is obtained in the sheet surface, and thereafter the panel with a relief pattern is painted in the painting line 3 and 4, whereby the different sides of the relief pattern will obtain different tones, and thus the color of the surface will vary, depending on the angle from which it is viewed. In this painting, conventional latex paints can be used, since the paint does not have to undergo pressing. On the other hand, the panel can also in this connection be first painted by the method according to the invention, and thereafter a relief pattern is formed also in the press, in which case the relief pattern may be the same as the pattern in the painting or different from it. When the abovementioned preferred paint is used, a hot pressing must be performed on the pulp sheet or pulp web after the painting, so that the starch sizes present in the paint will cook in the press and a sizing effect will be achieved.

In another embodiment of the invention, objects dipped in a coloring substance, for example straws of grass, may be placed on to the sheet before the pressing step, in which case the object will form a colored pattern on the panel surface. It is also possible to apply mica onto the sheet surface, whereby a metallic sheen is obtained.

In the method according to the invention it is indispensable to use a paint which will not adhere to the polish patterns of the press. Conventional latex paints are usually not suitable for this purpose. Therefore it is necessary to use a paint which is suitable for use in connection with the hot-pressing step of the method according to the present invention.

The principal component of the preferred coloring substance used in the method according to the invention is a chalk slurry having a solids content of approximately 65 %. The adhesive used for fixing the pigments to the panel surface is an uncooked starch, for example barley or potato starch, mixed with water. When the panels are heat-treated in the pressing step, the adhesive substances present in the wood itself will fix the surface so that the chalk will remain on the panel surface and will not penetrate it. In the hot press the starch present in the coloring substance cooks, and a sizing effect is obtained. Thus the preferred paint may be used where hot treatment is carried out. The temperature of the press is approximately 200 °C. At such a temperature the use of conventional latex paints is in general impossible.

The coloring substance preferably used in the method according to the invention contains chalk slurry, starch, and pigment. Chalk slurry is obtained as an industrial byproduct, and therefore it is economical. It is also possible to use dry chalk and to slurry it in water. The starch used may be, for example, potato or barley starch. When the coloring substance is being prepared, the starch is mixed with cold water and the starch slurry is added to the mixture of water and starch. The mixture must be stirred, since both starch and chalk tend to settle out.

The tone of the coloring substance is obtained by using various pigments. For example, Bayer's Levanyl color pigment pastes can be used. The amount of pigment is dependent on the desired degree of darkness of the color tone, but in general a very small amount of pigment will suffice for producing the color.

The composition of the paint mixture may vary within wide limits, depending on the targeted use. For example, a composition containing 0.5 l of a chalk slurry having a solids content of 65 %, 0.45 l of water, and 0.07 kg of barley starch has been found usable. The amount of starch depends, among other things, on the type of starch used.

By the method according to the invention, panels, pulp sheets or pulp webs are obtained the three-dimensional surface pattern of which may vary within very wide limits. These sheets or webs may be used, for example, in the packaging industry or for advertising and decorative purposes.

## Claims

1. A method for producing a three-dimensional surface effect on a panel, a pulp sheet or a pulp web, **characterized** in that a relief pattern or roughness is produced in the surface of the panel, pulp sheet or pulp web, whereafter a coloring substance or coloring substances is/are sprayed onto the surface of the rough-surfaced or relief-patterned panel, pulp sheet or pulp web from one or more directions, at an angle of less than 90 degrees, and after the spraying of the coloring substance or substances the pulp sheet or pulp web is pressed flat, or after the spraying of a coloring substance or substances a relief pattern is formed in the surface of the pulp sheet or pulp web in connection with the pressing.

2. A method according to claim 3, **characterized** in that the relief pattern is in accordance with the painted pattern or differs from it.

3. A method according to claim 1, **characterized** in that the relief pattern is produced by means of a roll.

4. A method according to claim 1, **characterized** in that the relief pattern is produced by means of an upper wire unit.
